

3,145,133  
**POLYAMIDE FILAMENT**

Bruce Arlyn Barton, Waynesboro, Va., assignor to E. I. du Pont de Nemours and Company, Wilmington, Del., 5 a corporation of Delaware  
No Drawing. Filed Dec. 21, 1962, Ser. No. 246,369  
8 Claims. (Cl. 161—168)

This invention relates to synthetic textile fibers and more particularly to the production of crimpable filaments having a high degree of crimp reversibility. 10

It is known in the art that drawn, composite filaments containing eccentric, differential shrinkage components, either in a side-by-side or a sheath-core relationship, develop a helical crimp when boiled off. Although such filaments have contributed substantially to the production of fabrics of improved aesthetics, further improvements are desired, particularly with respect to the bulk, covering power and handle of the fabrics. 15

Additionally, crimped composite fibers having the characteristic of decreasing the amount of crimp when exposed to a swelling agent and reverting to the original crimp upon removal of the swelling agent have been disclosed by Breen in U.S. 3,038,236. Although such crimp reversibility is responsible for some improvement in fabric bulk and covering power, the need for additional improvements is apparent, particularly with regard to the low crimping force exhibited by known high modulus, hydrophobic, composite fibers. 20

It is accordingly the most important object of this invention to provide an improved, reversible crimp filament characterized by a substantial increase in crimping force. A corollary objective is to provide a crimpable fiber, the use of which facilitates production of fabrics having improved bulk, covering power and handle. 25

These and other objectives are accomplished in a drawn, crimpable, composite filament including at least two continuous, adherent, polyamide components which are adapted to shrink differentially and thereby crimp as the filament first cools from a temperature of about 230° C. Thereafter, one of the components elongates reversibly and the other shrinks reversibly during each of several heating-cooling cycles. This novel combination of properties insures a crimped length contraction of at least 15% under a load of 0.0015 gram/denier each time the filament is cooled from 230° C. 30

Such a filament is prepared by melt extruding at least two components either in a side-by-side or a sheath-core relationship, the first component having, when extruded and drawn separately, a reversible thermal expansion at 230° C. of at least 0.75%. This component is a fiber-forming polyamide prepared from an aliphatic dicarboxylic acid and p-xylylene diamine (PXD) or a mixture of diamines containing at least 75% PXD. As noted previously, the other component, when extruded and drawn separately, shrinks reversibly during a similar heating-cooling cycle. The first component has a substantially greater initial shrinkage capacity and is thus the load-bearing component. 35

It has been found that crystalline, oriented filaments from the fiber-forming PXD polymers undergo reversible expansion to a high degree when the filament is heated. Thus, when the PXD polymer is used in a two-component filament with another polyamide which not only has a lower shrinkage but also the capability of shrinking reversibly in subsequent heating-cooling cycles, that filament exhibits a high degree of "squirm," i.e., a loss and gain of crimp when a fabric produced therefrom is subjected to repeated heating-cooling cycles. These factors 40

result in the development of improved bulk, covering power and handle in the fabric. 45

**EXAMPLE I**

The salt of p-xylylene diamine and azelaic acid is made by preparing an 11% by weight solution of azelaic acid in methanol in a stainless steel container and adding an equimolar quantity of p-xylylene diamine in the form of a 67% by weight solution in methanol while stirring the solution rapidly. The stirring is then reduced to a moderate rate and continued for 30 seconds after which the container is blanketed with nitrogen and allowed to stand without agitation for 3 hours. The mixture is then agitated for 5 minutes after which the salt is filtered off, washed with methanol and dried in a vacuum oven at a temperature of 80° C. for 60 hours. 50

The above salt, in the amount of 10,000 grams, is charged into an autoclave together with 10,000 grams of water, 30 grams of acetic acid and 125 grams of p-xylylene diamine. The autoclave is purged with nitrogen and heated rapidly to a temperature of 210° C. When the temperature reaches 200° C., 133 grams of 20% titanium dioxide delusterant slurry is added with agitation. After the temperature reaches 210° C., the temperature and pressure are maintained for 1 hour. The temperature is then raised to 250° C. and the pressure to 300 p.s.i. over a period of 30 minutes, after which the temperature is raised to 285° C. and the pressure reduced to atmospheric over a period of 45 minutes, this condition being maintained for an additional period of 2 hours. 55

The polymer (PXD-9) is discharged from the autoclave and cut into flake as described in U.S. 2,289,774. The flake has an inherent viscosity of 0.72. 60

Polyhexamethylene adipamide (6-6 nylon) flake having a relative viscosity of 45 is prepared in the conventional manner. The 6-6 and PXD-9 flakes are melted separately in screw melters and then extruded in continuous, adherent, side-by-side relation from 34 holes in a spinneret of the type shown in FIG. 6 of U.S. 2,931,091 to produce composite filaments in which the two components are present in an approximately 1:1 weight ratio. The freshly spun filaments are quenched by passing air transversely across the bundle, as described in U.S. 2,273,105, and then wound into a package in the conventional manner. The yarn is subsequently drawn, as shown in U.S. 2,289,232, on a draw-twister, the draw ratio being 4. The denier of the final yarn is 70. 65

When the crimpable, composite yarn is oven heated in a relaxed state at 230° C. and cooled, an excellent helical crimp develops with the PXD-9 component on the inside of the helix. The reversible loss and gain of crimp or "squirm" in the yarn is measured by heating the dry, crimped yarn to 230° C. and again cooling to 25° C. The percent squirm under no restraint and under various degrees of slight restraint is determined by suspending crimped samples in a closed, electrically heated tube, measuring their length, heating the samples to 230° C., measuring, cooling to 25° C. and again measuring sample lengths. The squirmability reported in Table I is calculated from the various measurements. Where reported, the indicated loads were attached to the free ends before heating the crimped samples to 230° C. For comparison, results obtained with several other two-component yarns are also shown, fiber A being a two-component yarn in which one component is poly(m-xylylene adipamide) (MXD-6) and the other component is 6-6 nylon, fiber B a two-component yarn in which one component is poly(ethyleneterephthalate) and the other component is 6-6 nylon and fiber C a two-component yarn in which one component is the polymer derived from bis-p-amino-cyclohexylmethane and azelaic acid and the other component is 6-6 nylon. 70

3  
Table I

| Load, g.p.d. | Percent Squirm |        |       |        |
|--------------|----------------|--------|-------|--------|
|              | 0              | 0.0005 | 0.001 | 0.0015 |
| PXD-9/6-6    | 55             | 37     | 25    | 21     |
| Fiber A      | 32             | 17     | 11    | 6      |
| Fiber B      | 48             | 13     | 5     | 3      |
| Fiber C      | 13             | 10     | 7     | 3      |

When swelled and dried according to the procedures disclosed by Breen in U.S. 3,038,236, the crimped PXD-9/6-6 composite filament elongated and contracted by only 18% under no load. Under a load of 0.001 g.p.d., only a 12% squirm was observed.

When the PXD-9 component is extruded and drawn separately, the yarn shrinks 17% when initially heated to 230° C. and then cooled to 25° C. Thereafter, the yarn expands 1.3% in length upon heating to 230° C. and contracts to its original shrunk length upon cooling to 25° C. The 6-6 component, when treated in this fashion, shrinks 12% initially and, upon subsequent heating and cooling, shrinks 1.8% and then elongates to its original length. Repeated heating-cooling cycles show these thermal expansion and shrinkage characteristics to be permanently reversible.

Uncrimped yarn, prepared as described above, is crimped at 232° C. and knit tubing is prepared from the yarn in the conventional manner. The tubing is repeatedly oven heated to 230° C. and cooled to room temperature. After three cycles, a substantial improvement in bulk, covering power and hand is noted. By comparison, tubings knitted from crimped fibers A, B and treated similarly show far less improvement.

#### EXAMPLE II

Two-component, 30 denier, 10 filament, PXD-9/6-6 yarn is prepared as described in Example I. The drawn, uncrimped yarn is coned and knitted into a 32 inch, 28 gauge, 15 quality jersey tricot fabric which is subjected to a conventional scour, oven dried at 120° C. and heated at 210° C. in a relaxed state to develop crimp. After cooling, the fabric has considerable bulk because of the crimping action. A portion of the bulked fabric is heated repeatedly to 230° C. followed by cooling to room temperature. After three cycles, it is further improved in covering power, bulk and hand.

#### EXAMPLE III

Following the general procedure of Example I, 70 denier, 34 filament, side-by-side, two-component yarns are prepared with 6-6 nylon as one component and various PXD polymers and copolymers as the other component. These included p-xylylene adipamide, the copolymer containing 90% p-xylylene azelamide and 10% m-xylylene azelamide and the copolymer containing 75% p-xylylene azelamide and 25% m-xylylene azelamide. The two-component yarns containing other PXD polymers and copolymers exhibit about the same reversible expansion when heated to 232° C. as the two-component yarn containing PXD-9 (Example I). When these yarns are knitted into fabrics, the results are substantially the same as found in Example I.

As indicated in the foregoing examples, the crimpable yarn of this invention may be utilized in fabrics, particularly knit fabrics, to produce a very desirable improvement in bulk, covering power and hand.

The crimped fibers of this invention are unique in that the load-bearing component exhibits a high degree of thermal expansion. Consequently, the fibers not only lose crimp when heated but also have the ability to contract or re-crimp on cooling against restraining forces which prevent prior art fibers from contracting to such an extent. As shown in Table I, a two-component filament (fiber C) in which the high shrinkage component is 6-6

nylon and the other component is polyethylene terephthalate, i.e., a fiber of the same composition disclosed in Examples II and III of U.S. Patent No. 3,038,236 to Breen, shows about the same retraction under no restraint as the fiber of this invention but, under a load of 0.001 g.p.d. (a degree of restraint which exists in fabrics), the instant fiber has a five-fold advantage. Even in comparison with a two-component fiber from 6-6 nylon and an MXD polyamide (fiber A, Example I), the fibers of this invention show a two-fold advantage.

To obtain the results disclosed herein, one component of the composite filament should have a reversible thermal expansion of at least 0.75%, preferably 1.0%, based on the extended length of the fiber before expansion, when heated to 230° C. and subsequently cooled to 25° C. under a restraint of 0.001 g.p.d., i.e., the polymeric material in that one component, when extruded and drawn separately, must expand at least 0.75% when heated and then contract to substantially its shrunk length under a restraining load of 0.001 g.p.d. This component must also have a higher shrinkage than the other components in the fiber when initially heated to 230° C. and then cooled. In this connection, it should be noted that the high shrinkage polyamide components disclosed by Breen, e.g., 6-6 nylon in Examples II and III of U.S. 3,038,236, are not thermally expansible. The preferred polymeric materials for use as the high shrinkage component are those derived from p-xylylene diamine and aliphatic dicarboxylic acids. Suitable aliphatic acids include adipic acid, suberic acid, sebacic acid, undecan-dioic acid, and dodecan-dioic acid. A mixed acid-containing up to 25% of another aliphatic acid or of a non-aliphatic acid such as isophthalic acid or terephthalic acid may be employed. Copolymers containing up to about 25% of another diamine may also be employed.

The other component or components in the fiber may consist of any other synthetic linear fiber-forming polyamide having a relatively low initial shrinkage upon cooling from a temperature of about 230° C. As against thermal expansibility, this component should shrink reversibly when subsequently heated and cooled. Suitable polymers include 6-6 nylon, 6 nylon, polyoctamethylene oxamide, polyhexamethylene sebacamide and various copolymers.

In order to obtain the improvements of this invention, the thermally expansible component must have the higher initial shrinkage, i.e., it must be the load bearing component in the crimped fiber. In order to accomplish this, it must be prepared from a polymer having a molecular weight in the fiber-forming range. If lower molecular weight polymers are employed, this component does not have the higher shrinkage of the two components and the desired product is not obtained.

In order to perform satisfactorily, the fibers of this invention must, of course, be drawn and the orientation so produced must be substantially retained after the heating and cooling treatment which is necessary to produce the requisite thermal "squirm." Undrawn fibers or fibers which become deoriented on heating (e.g., fiber C, Example I) are not satisfactory.

Having thus described the invention, what is claimed as new and desired to be secured by Letters Patent is:

1. A drawn, crimpable, composite filament comprising two continuous, adherent, polyamide components adapted to shrink differentially and thereby crimp as the filament first cools from an elevated temperature, one of said components being adapted to elongate reversibly and the other to shrink reversibly in subsequent heating-cooling cycles, said one component being of fiber-forming molecular weight and also having an initial shrinkage potential relatively higher than that of the other component.

2. The crimpable filament of claim 1 wherein said one component comprises the polyamide prepared from p-xylylene diamine and an aliphatic dicarboxylic acid.

3. The crimpable filament of claim 1 wherein said one component consists essentially of the polyamide prepared from p-xylene diamine and an aliphatic dicarboxylic acid.

4. The crimpable filament of claim 3 wherein said other component consists essentially of a polyamide selected from the group consisting of polyhexamethylene adipamide, polycaproamide, polyoctamethylene oxamide, polyhexamethylene sebacamide and copolyamides thereof.

5. A drawn, crimpable, composite filament comprising continuous, adherent components of fiber-forming poly-*p*-xylylene azelamide and polyhexamethylene adipamide.

6. A drawn, crimped, composite filament comprising two continuous, adherent, polyamide components, one of said components being adapted to elongate reversibly and the other to shrink reversibly in repeated heating-

cooling cycles, said one component being of fiber-forming molecular weight, said filament being characterized by a crimped length contraction of at least 15% upon cooling from 230° C. under a load of 0.0015 gram/denier.

5 7. A fabric containing a plurality of filaments of claim 6.

8. A fabric containing crimped, composite, squirmable filaments each comprising continuous, adherent components of fiber-forming poly-*p*-xylylene azelamide and polyhexamethylene adipamide, said filaments being characterized by a crimped length contraction of at least 15% upon cooling from 230° C.

References Cited in the file of this patent

UNITED STATES PATENTS

15 2,931,091 Breen \_\_\_\_\_ Apr. 5, 1960